

Nov. 6, 1945.

N. J. PENNING

2,388,568

SEALING COMPOSITION

Filed March 4, 1942



INVENTOR  
Nicholas J. Penning  
BY *Maurice Brown & Co.*  
ATTYS

## UNITED STATES PATENT OFFICE

2,388,568

## SEALING COMPOSITION

Nicholas J. Penning, Milwaukee, Wis.

Application March 4, 1942, Serial No. 433,367

11 Claims. (Cl. 260—750)

Crown bottle caps, those caps which are applied to beer and soft drink bottles, require a sealing member compressed between them and the rim of the bottle in order to effectuate a seal. These sealing members or seals, as they are commonly called, have conventionally been formed of a thin disc of cork or cork composition faced on the side exposed to the bottle contents with a disc of tin foil or the like, called a spot.

These seals have never been completely satisfactory because of a tendency for the formation of mold beneath the spot. They have, however, been more satisfactory than anything else commercially available. At the present time, in fact, even these seals can hardly be said to be commercially available in view of the material shortage, especially in tin foil.

One reason that no other seal has been as satisfactory is because of the difficulty of avoiding the impartation of taste or odor to the contents of the bottle. Even tastes or smells which most people would not notice would be noticed by enough people so that the reputation of a product, particularly in the case of a beverage, would be impaired. Another factor that must be taken into consideration is the pressure with which the caps are conventionally applied. A material which is too soft will flow under this pressure with the result that, when the pressure is released, there may be leakage. On the other hand, it is necessary for the material to be yieldable in order to effectuate a satisfactory seal. Another requirement is that the material should not be tacky—it should not adhere to the glass.

According to the present invention, the various requirements have been met by the use of a rubber and wood flour composition substantially free from any ingredients which will impart taste or odor to the contents of the bottle and which can be manufactured at a sufficiently low cost to be commercially practical. Of course, the price must be low enough to be practically insignificant in relation to the total cost of the bottled beverage. The proper consistency is obtained without the cost of vulcanization by heat by using a relatively high content of filler which is largely wood flour and by mixing the rubber and filler in such a way as to leave a large proportion of the natural rubber globules unbroken.

Additional advantages and objects of the invention will be apparent from the following description and from the drawings, which show in cross section and more or less diagrammatically

a bottle cap applied to a bottle and embodying the seal of the present invention.

Although only one form of bottle cap and seal have been illustrated, the form of cap being that for which the present invention is particularly designed, it will be evident that other forms of caps can be used and that wide departures may be made from the preferred composition of the seal while retaining at least some of the advantages of the present invention.

Full details of the preferred composition and its treatment are given in accordance with the requirements of R. S. 4888 but are not intended for limitation of the scope of the invention except as required by the prior art.

In the drawing the bottle cap 11 is applied to a bottle 12 in a conventional manner and includes a conventional crimped flange which exerts a pressure on the underside of an annular bead 14 at the mouth of the bottle to hold the cap firmly in place. Hermetic sealing of the bottle is effectuated by a seal 16 with which the present invention is particularly concerned. It may be inserted loose or cemented with adhesives heretofore used in bottle caps, as albenum for example.

As seen from the drawing, the seal 16 may comprise a single layer. As previously mentioned, it is necessary for the seal to be yieldable to effectuate the seal and, as a matter of fact, it is also necessary for it to be resilient so that after the pressure used in applying the cap is released the seal will tend to expand and continue to exert a pressure against the bottle. Various rubber compositions have been tried in the past but have all been found to be unsatisfactory, either because they lacked the right consistency or because they imparted taste to the contents of the bottle.

According to the present invention, the preferred composition and method of formation of the seal 16 are as follows, the proportions being by weight throughout:

|                          | Parts |
|--------------------------|-------|
| Pale crepe rubber        | 25    |
| Leached maple wood flour | 75    |

The wood flour may be leached by boiling for about ten minutes in several times its volume of a good grade of water, allowing the wood flour to settle, decanting the water therefrom (or otherwise separating the flour from the liquid), and drying the flour.

The rubber and flour are mixed by first applying the rubber to a standard rubber mill having its rolls heated to approximately 300° F. and ap-

plying the wood flour thereto as soon as the rubber begins to level out, which will usually be in about one minute. The mixture should be removed from the mill as soon as the wood flour has been well incorporated and uniformly mixed through the rubber, which will usually be within four minutes more. After cooling, the mixture is then calendered, the rolls of the calender being warm, according to conventional practice, a temperature of 150° F. being satisfactory.

It will be evident that wide departures can be made from the foregoing formula and treatment. Some departures will have no deleterious effect. Others will cause a failure to obtain the full advantages of the invention but will still yield a satisfactory sealing composition. For example, considerable departure may be made from the milling temperature stated, but best results are obtained by having the temperature approximately as high as 300° F., since this permits a rapid mixing of the rubber and wood flour without greatly breaking down the rubber. In other words, a substantial proportion of the rubber globules are retained unbroken in their original state. For those not skilled in the art, it may be noted that rubber latex is formed of very minute rubber globules in an aqueous suspension, some resins and proteins being present in addition to the rubber molecules and water. In the course of forming pale crepe from this latex, most of the water is removed and a considerable proportion of the other non-rubber ingredients are washed out, and it is probable that some of the rubber globules are broken. The brief mixing on the hot mill preferred, by maintaining as many as possible of the globules intact, results in a finished product which has the proper consistency without vulcanization.

In place of wood flour, any other ground fibrous cellulose may be used—for example, ground corn-cobs or corn stalk pith. For many uses, however, as for example with beer, care must be taken to choose one which will not impart a taste to the contents of the bottle. I have determined that, considering availability, the very best from a wide variety of possibilities is rock maple ground to a flour, and that it is improved by the leaching process mentioned. Quite a few others might be found that would be satisfactory for any given purpose, especially if leached to remove taste-imparting or taste destroying ingredients. Of course, non-cellulosic fibrous materials could also be used if they meet the other tests. They should, however, be in very small particles comparable to the particle size of wood flour, rather than in long fibers. It is believed to be desirable for the small particles to themselves be composed of a plurality of extremely fine fibres so that they will tend to interlock with one another and prevent flowing of the finished product under the pressure of capping the bottle.

It is not necessary that all of the filler be of this fibrous nature. Fairly satisfactory results have been obtained with only 25% of the total weight composed of wood flour, the remainder of the filler being a mineral such as clay. The seal should not be tacky enough to stick to glass and hence total filler content should be about 60% to about 80% of the total weight if all wood flour, or the equivalent thereof in reducing tackiness.

Although pale crepe rubber is preferred, any other rubber or similar rubber-like substance, including synthetic rubber, which will not impart a taste or smell, and which will yield the proper consistency of the finished product may be used. The consistency should be similar to that of cork,

except that it need not snap back as quickly after pressure is released. Among the synthetic rubbers, the buna types seem best, having the least odor and being more than stiff enough.

Although seals made in accordance with the foregoing disclosure are entirely satisfactory for beverages, if they are to be used for hydrocarbons, such as gasoline and petroleum oil, they can be very readily made substantially immune thereto by subjecting them or the sheet from which they are cut to a half-hour curing with the vapor of a small amount of sulphur chloride in a closed container at room temperatures, a temperature of about 70° F. having been specifically found to be suitable.

A suitable substance may be included if desired for rendering the individual wood flour particles impervious to moisture. One suitable substance is that known as "Flex Wax C" sold by Glyco Products Company of New York city. It is non-toxic and insoluble in alcohol and in water and melts to a liquid at about 145° F. and does not affect the taste or smell of beverages in contact therewith. The wax may further be identified as that specific wax disclosed in the publication "Chemicals by Glyco," copyright 1940, especially at page 34. Properties of this wax include the following: Color—tan, luster—dull, flash point—257° C., specific gravity at 20° C.—.820, soluble in hot tallow oil, hot naphtha, hot mineral oil, and hot vegetable oil, the solution in vegetable oil gelling when cold. It is mixed simultaneously with the wood flour and rubber and is substantially sorbed (probably absorbed) by the flour. Five per cent of the weight of the mixture to which it is added is preferred, but from 3 to 20% may be used advantageously. Being sorbed, it has little effect on the proportions that should be used aside from the wax.

A seal produced in accordance with the foregoing disclosure, even without the treatment with sulphur chloride, produces a more satisfactory seal than any known before this invention. It is adequately impervious to liquids and gas; it is immune to alcoholic and aqueous solutions; it imparts no detectable taste or odor to such solutions or beverages; and it has the proper consistency including resistance to flow and resiliency. Furthermore, it can be made at a very low cost because of the fact that its major ingredient, wood flour, is very inexpensive and the further fact that it requires no vulcanization and hence may be made simply by brief mixing and calendering. In the form in which the composition is surface-vulcanized with sulphur chloride, it can be used in contact with hydrocarbon solvents. For this purpose it will not ordinarily need to be free from taste or odor imparting ingredients. When vulcanized throughout with sulphur chloride, it is suitable for numerous other uses where it may be subjected to pressures considerably greater than the conventional bottling pressures.

I claim:

1. A bottle-sealing composition consisting essentially of 25 parts by weight of pale crepe rubber, and approximately 75 parts of rock maple wood flour thoroughly mixed therein; said rubber being substantially unbroken-down, and said compound having such a consistency that it will yield resiliently but will not appreciably flow under conventional bottle-sealing practices.

2. A bottle cap comprising a disc of metal having a crimped flange therearound and a pre-

formed sealing member inserted therein formed of the composition set forth in claim 1.

3. The method of making bottle seals, which consists essentially in boiling rock maple wood flour in water, decanting the water, applying pale crepe rubber to a hot mill, adding the wood flour to the rubber as soon as the rubber begins to level out until the wood flour is about 75% of the total by weight, removing the mix as soon as the wood flour has been well incorporated, calendering the mix, and cutting the seals from the resulting sheet.

4. A composition consisting essentially of unvulcanized rubber, and a filler consisting mainly of maple wood flour, with the filler comprising 60-80% of the weight.

5. A sealing composition consisting essentially of unvulcanized rubber matrix and a filler in a proportion equivalent in eliminating tackiness to 60% by weight of wood flour, a portion of the filler, comprising at least 33% of the matrix weight, comprising maple wood flour.

6. A sealing composition consisting essentially of unvulcanized rubber matrix and a filler in a proportion sufficient to prevent the rubber from 25 sticking to glass, a portion of the filler, com-

prising at least 33% of the matrix weight, comprising maple wood flour.

7. A bottle sealing disk having the composition set forth in claim 6.

8. A bottle-sealing composition consisting essentially of 25 parts by weight of pale crepe rubber, and approximately 60 to 80 parts of maple wood flour thoroughly mixed therein, the said rubber being substantially unbroken-down; and 10 said compound having such a consistency that it will yield resiliently but will not appreciably flow under conventional bottle-sealing practices.

9. A bottle-sealing disc formed of the composition set forth in claim 8.

15 10. A bottle-sealing composition consisting essentially of pale crepe rubber and at least twice the weight thereof of maple wood flour thoroughly mixed therein; the said rubber being substantially unbroken-down, and said compound having such a consistency that it will yield resiliently but will not appreciably flow under conventional bottle-sealing practices.

11. A bottle-sealing disc formed of the composition set forth in claim 10.

NICHOLAS J. PENNING.